

# UNITED STATES PATENT OFFICE.

WILLIAM L. GEDDES, OF PHILADELPHIA, PENNSYLVANIA, ASSIGNOR TO MAC-  
ANDREWS & FORBES COMPANY, OF CAMDEN, NEW JERSEY, A CORPORATION  
OF NEW JERSEY.

## LICORICE-ROOT-FIBER BOARD.

1,143,621.

Specification of Letters Patent. Patented June 22, 1915.

No Drawing.

Application filed April 9, 1914. Serial No. 830,739.

To all whom it may concern:

Be it known that I, WILLIAM L. GEDDES, a citizen of the United States, residing at Philadelphia, in the county of Philadelphia and State of Pennsylvania, have invented new and useful Improvements in Licorice-Root-Fiber Board, of which the following is a specification.

This invention relates to the preparation 10 of artificial board or box board, which has many industrial uses.

One of the objects of the invention is to produce a board from the fibrous residue of licorice root by a very simple process, which 15 is of superior quality and of a durable and nearly uninflammable nature.

Another object of the invention is to produce a board which will be of very uniform texture and homogeneous in character.

20 A further object of the invention is to produce a board which can be very effectively waterproofed.

The invention resides in the application 25 of pulp made from spent licorice root by a process to be described hereinafter, and in the products resulting from the application of the process. (Spent licorice root is the waste product from the manufacture of licorice extract.)

30 I have discovered that a pulp formed from spent licorice root has highly cohesive properties when formed into board, and that a board formed of this material is of superior quality.

35 In practising my invention I mix a caustic substance, such as caustic soda, with the spent root for the purpose of removing the resinous and non-cellulose constituents and cleaning the fibers, and the resulting pulp is 40 afterward washed to remove the alkaline solution carrying these constituents. The pulp is then passed in the usual manner through the beater and Jordan engine, and thence to the board machine, where it is formed into 45 sheets. The sheets which come from the board machine are suitable for use in forming containers or as jacquard board, or for other purposes. In order to produce such boards as wall board and panel board I prefer to connect a plurality of superimposed 50 sheets together by a suitable adhesive preferably silicate of soda. After applying the adhesive the sheets are pressed together and

the thickness of the board which is desired is determined by the number of sheets so 55 connected together. The board resulting from this process is perfectly homogeneous as substantially all the constituents of the root have been removed except the cellulose.

For this reason the board absorbs sizing and 60 other waterproofing materials easily, and with complete uniformity. For this and other reasons this board is far superior to boards having a heterogeneous character,

such as boards formed of ground wood, 65 straw, waste papers, or other materials which have a variety of different chemical constituents.

This board is also nearly fireproof for the reason that it is nearly devoid of the inflammable resinous matters such as are 70 contained in board made from ground wood.

In making wall board from the sheets of this spent licorice root pulp a fireproof cement may be used to connect the sheets together. The treatment of the fiber with the 75

caustic substance renders it absolutely sterile, and on this account no bacterial or mold growth will take place and vermin will not be attracted to the board. Other boards,

such as are made from pulp composed of the 80 mixture of newspapers, rags, etc., are favorable media for bacterial culture, mold growth, or for attack by vermin. Boards

made from ground wood are even more susceptible to vermin attack than the original 85 wood from which they were made. The board made from spent licorice root pulp

fiber is difficult to ignite and the flames tend to die out, simply leaving the cellulose 90 smoldering. A board formed from spent licorice root pulp is relatively stiff and has a relatively high tensile strength. It is also tough and relatively more durable than other artificial boards. It is also a better

non-conductor of heat and is an effective 95 sound deadener, which is desirable when the board is used as a wall board. On account

of its greater stiffness and hardness a thinner board of this kind can be used as compared with the ordinary "news" or "chip" 100

board to fill the ordinary requirements for which so called box board can be used, thus effecting a marked economy to the consumer

by reason of the greater sheet area for a given weight of material; and if a quantity 105 of spent licorice root pulp is mixed with

other pulp or pulps the qualities of the product are materially improved thereby, and such mixture when made into board tends to acquire many of the superior qualities of spent licorice root board.

What I claim is:—

The process of forming artificial board, which consists in treating spent licorice root with a caustic substance to remove the resin and other non-cellulose constituents, wash-

ing the caustic substance from the pulp thereafter and forming the pulp into sheets.

In testimony whereof I have hereunto set my hand in presence of two subscribing witnesses.

WILLIAM L. GEDDES.

Witnesses:

W. E. RANSOM,  
FRANK J. MAGINNIS.